



US005998121A

# United States Patent [19]

Southby et al.

[11] Patent Number: 5,998,121

[45] Date of Patent: Dec. 7, 1999

[54] **PHOTOGRAPHIC ELEMENT WITH SILVER HALIDE EMULSION LAYER OF LOW DEVELOPABILITY AND HAVING AN ASSOCIATED HIGH DYE-YIELD COUPLER**

[75] Inventors: **David T. Southby; James T. Kofron**, both of Rochester; **Robert J. Newmiller**, Webster, all of N.Y.

[73] Assignee: **Eastman Kodak Company**, Rochester, N.Y.

[21] Appl. No.: **08/729,930**

[22] Filed: **Oct. 15, 1996**

## Related U.S. Application Data

[63] Continuation-in-part of application No. 08/250,742, May 27, 1994, abandoned.

[51] **Int. Cl. 6** ..... **G03C 7/333**; G03C 7/18

[52] **U.S. Cl.** ..... **430/543**; 430/226; 430/359; 430/557; 430/958

[58] **Field of Search** ..... 430/543, 226, 430/958, 359, 557

[56]

## References Cited

### U.S. PATENT DOCUMENTS

|           |         |                      |         |
|-----------|---------|----------------------|---------|
| 4,711,837 | 12/1987 | Ichijima et al. .... | 430/958 |
| 4,840,884 | 6/1989  | Mooberry et al. .... | 430/543 |
| 4,842,985 | 6/1989  | Ono et al. ....      | 430/226 |
| 5,447,819 | 9/1995  | Mooberry et al. .... | 430/226 |
| 5,457,004 | 10/1995 | Mooberry et al. .... | 430/226 |

*Primary Examiner*—Richard L. Schilling  
*Attorney, Agent, or Firm*—Arthur E. Kluegel

[57]

## ABSTRACT

The photographic element of the invention provides a support bearing at least one photographic silver halide emulsion exhibiting low developability and having associated therewith at least one high dye-yield coupler that releases a dye or dye precursor having an electrically neutral dye chromophore. The invention also encompasses a process for forming an image in an element in accordance with the invention.

**13 Claims, No Drawings**

## 1

**PHOTOGRAPHIC ELEMENT WITH SILVER HALIDE EMULSION LAYER OF LOW DEVELOPABILITY AND HAVING AN ASSOCIATED HIGH DYE-YIELD COUPLER**

**CROSS REFERENCE TO RELATED APPLICATIONS**

This application is a Continuation-in-Part of application Ser. No. 08/250,742, filed May 27, 1994, now abandoned.

**FIELD OF THE INVENTION**

This invention relates to a photographic element containing a photographic silver halide emulsion layer exhibiting low developability and having associated therewith a high dye-yield coupler.

**BACKGROUND**

This invention involves the use of an image dye-forming coupler which releases a dye or dye precursor as the coupling off group. These are so-called "High Dye-Yield" (HDY) couplers because they form two molecules of dye for each molecule of coupler which is consumed.

Useful high dye-yield couplers have been disclosed by Mooberry and Singer in U.S. Pat. No. 4,840,884. (The '884 patent) Such couplers react with oxidized color developer to form one dye and in doing so release a precursor of a second dye having a neutral dye chromophore. In accordance with the patent, the new couplers described therein enable lower concentrations of silver halide in the photographic element without lowering image quality.

Among the desirable features of photographic elements are high speed (good low-light sensitivity) and low fog (non-imagewise development). Silver halide emulsions are prepared to have the most advantageous combination of high photographic speed and low fog development. This is done by design using for example, iodide content and distribution, grain size and morphology and by the degree of finishing in which the type or level of sensitization and additives which decrease fog formation are varied. Thus, there are various ways of controlling fog each having its own effect on speed. At the most advantageous speed/fog position the emulsion can be used most efficiently for imaging. However, at this speed/fog position, the emulsion may not give sufficient developed silver and so may not give sufficient dye formation (Dmax and density gradient) when coated with an imaging coupler, to make it useful in film embodiments.

In color negative processing in accordance with the Kodak Flexicolor C-41 process, the time of development (tod) is 3.25 minutes. As the tod is varied from 3.25 to 4.5 minutes both speed and fog will increase for an element given a step wedge exposure. If the emulsion is coated with an imaging coupler such that there is sufficient development at each tod to reach maximum dye density (Dmax), then, as tod is increased, the film contrast will increase along with the fog (read out as D<sub>min</sub>) until or unless the D<sub>min</sub> rises rapidly enough to suppress the contrast.

The region where the contrast and D<sub>min</sub> do not change substantially with changes in development time (around the 3.25 minutes used for conventional photographic elements) is the region of maximum efficiency for that coupler/silver combination.

High speed emulsions with high iodide contents are provided with addenda during finishing in a manner well-known in the art in order to sensitize the grains to obtain the desired high speed and contrast. This often leads to rela-

## 2

tively high D<sub>min</sub> values. Emulsions finished to have lower D<sub>min</sub> values typically have lower contrast but may have adequate speed. High-speed, high-iodide emulsions are, generally, low in developability.

5 High iodide content emulsions show lower contrast and often, when this deficiency is combined with inefficiencies in dye formation and dye covering power, need to be coated at higher levels than would lower iodide level emulsions, in order to get the desired contrast. This, of course, interferes with the properties of the element.

10 It is a problem to be solved to provide an emulsion that is associated with a particular type coupler and that, when finished to have low D<sub>min</sub> and contrast, gives a sensitometric response that is improved over that of a more developable emulsion having a conventional coupler associated therewith.

**SUMMARY OF THE INVENTION**

20 The photographic element of the invention provides a support bearing at least one photographic silver halide emulsion exhibiting low developability and having associated therewith at least one high dye-yield coupler that releases a dye (or dye precursor) having an electrically 25 neutral dye chromophore. The invention also encompasses a process for forming an image in an element in accordance with the invention.

30 The photographic element of the invention provides an emulsion which is finished to have low D<sub>min</sub> and low developability but which has an associated coupler which gives a sensitometric response that is improved over that of a more developable emulsion having a conventional coupler associated therewith.

**DETAILED DESCRIPTION OF THE INVENTION**

35 The invention provides a photographic element comprising a support bearing a light sensitive photographic silver halide emulsion layer wherein the layer has associated therewith a coupler capable of combining with oxidized developer to form a first dye, the coupler also containing a coupling-off group which is released during development to form a precursor of a second dye, the precursor having an electrically neutral dye chromophore bonded to a linking group selected from the group consisting of  $-\text{OC}(\text{O})-$ ,  $-\text{OC}(\text{S})-$ ,  $-\text{SC}(\text{O})-$ ,  $-\text{SC}(\text{S})-$ , and  $-\text{OC}(\text{R})-$  where R is substituted or unsubstituted alkyl or aryl;

40 45 50 55 55 wherein the amount of said coupler associated with the layer and the amount of silver in the layer is such that the molar ratio of the dye formable from the coupler to the silver contained in the layer is less than 1.0 and the coupler levels are each below 1 g/m<sup>2</sup>. It is desirable but not essential that the second dye has a calculated logarithm of its neutral partition coefficient (ClogP) in the range of 3.5 to 5.5.

55 60 The dye forming coupler of the invention has the general formula:



65 where COUP is the parent group of the coupler capable of reacting at the coupling position with oxidized color developer to form a first dye, T is one or more optional timing groups with m=0 to 2, L is a particular linking group, and DYE is a second dye.

COUP is the parent portion of a coupler that is capable of coupling with oxidized developer to form a dye. As described more fully hereafter, the dye may be of any desired color or may be colorless and if desired, it may be of the so-called universal type which washes out of the element during processing.

Image dye-forming couplers may be included in the element such as couplers that form cyan dyes upon reaction with oxidized color developing agents which are described in such representative patents and publications as: U.S. Pat. Nos. 2,367,531, 2,423,730, 2,474,293, 2,772,162, 2,895, 826, 3,002,836, 3,034,892, 3,041,236, 4,333,999, 4,883,746 and "Farbkuppler-eine LiteratureUbersicht," published in Agfa Mitteilungen, Band III, pp. 156-175 (1961). Preferably such couplers are phenols and naphthols that form cyan dyes on reaction with oxidized color developing agent.

Couplers that form magenta dyes upon reaction with oxidized color developing agent are described in such representative patents and publications as: U.S. Pat. Nos. 2,311, 082, 2,343,703, 2,369,489, 2,600,788, 2,908,573, 3,062,653, 3,152,896, 3,519,429, and "Farbkuppler-eine LiteratureUbersicht," published in Agfa Mitteilungen, Band III, pp. 126-156 (1961). Preferably such couplers are pyrazolones, pyrazolotriazoles, or pyrazolobenzimidazoles that form magenta dyes upon reaction with oxidized color developing agents.

Couplers that form yellow dyes upon reaction with oxidized color developing agent are described in such representative patents and publications as: U.S. Pat. Nos. 2,298, 443, 2,407,210, 2,875,057, 3,048,194, 3,265,506, 3,447,928, 4,022,620, 4,443,536, and "Farbkuppler-eine LiteratureUbersicht," published in Agfa Mitteilungen, Band III, pp. 112-126 (1961). Such couplers are typically open chain ketomethylene compounds.

Couplers that form colorless products upon reaction with oxidized color developing agent are described in such representative patents as: U.K. Patent No. 861,138; U.S. Pat. Nos. 3,632,345, 3,928,041, 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Pat. Nos. 1,939,231; 2,181,944; 2,333,106; and 4,126,461; German OLS No. 2,644,194 and German OLS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3-position may be employed. Couplers of this type are described, for example, in U.S. Pat. Nos. 5,026,628, 5,151, 343, and 5,234,800.

T is a timing group which, as indicated by the value range for m of from 0 to 2, may be absent or may represent one or two such timing groups. Such groups are well-known in the art such as (1) groups utilizing the cleavage reaction of a hemiacetal (U.S. Pat. No. 4,146,396, Japanese Applications 60-249148; 60-249149); (2) groups utilizing an electron transfer reaction along a conjugated system (U.S. Pat. Nos. 4,409,323; 4,421,845; Japanese Applications 57-188035; 58-98728; 58-209736; 58-209738); (3) groups utilizing the cleavage of imino ketals (U.S. Pat. No. 4,546,073); (4) groups that function as a coupler or reducing agent after the

coupler reaction (U.S. Pat. Nos. 4,438,193; 4,618,571); and (5) groups using an intramolecular nucleophilic substitution reaction (U.S. Pat. No. 4,248,962). The timing group to which the L-DYE group of the invention is optionally attached is any one which will permit release of the L-DYE group. Foregoing group (5) is not suitable as the group to release L-DYE but could serve as the first of a sequence of two timing groups. Other timing groups are generally suitable for releasing —L-DYE. Timing groups as described under (2) and the listed patents are most suitable. Generally these consist of a bond from COUP or another timing group to an oxygen atom which is bonded to a substituted or unsubstituted aromatic hydrocarbyl or heterocyclic ring at a location in conjugation with a methyl group on the ring which may optionally be substituted with one or two alkyl groups, where the methyl group is bonded to L-DYE or a second timing group. A typical such group based on an aromatic hydrocarbyl group has the formula:



wherein Z is selected from the group consisting of nitro, cyano, alkylsulfonyl; sulfamoyl ( $-\text{SO}_2\text{NR}_2$ ); and sulfamido ( $-\text{NRSO}_2\text{R}$ ) groups; R is hydrogen or a substituent such as alkyl; R¹, R¹¹ and R¹² are independently hydrogen or substituents that do not adversely affect the coupling and release reactions or the properties of the dyes formed thereby.

One example of such a group containing an aromatic heterocycle is:



where R⁹ through R¹² are independently hydrogen or substituents that do not adversely affect the coupling and release reactions or the properties of the dyes formed thereby.

L is a group which serves to connect COUP (or T, if present) to the second dye. L has a formula so as to permit —L-DYE or —(T)<sub>m</sub>—L-DYE to be cleaved from the coupler upon the coupler's oxidative coupling with color developer during development processing. COUP combines with the oxidized developer to form the first dye and the fragment —L-DYE or —(T)<sub>m</sub>—L-DYE is then freed from COUP. Suitable groups for L are  $-\text{OC}(\text{O})-$ ,  $-\text{OC}(\text{S})-$ ,  $-\text{SC}(\text{O})-$ ,  $-\text{SC}(\text{S})-$ , or  $-\text{OC}(\text{=NSO}_2\text{R})-$ , where R is substituted or unsubstituted alkyl or aryl. Such groups permit the cleavage of the fragment from COUP and are cleaved from DYE. U.S. Pat. No. 4,840,884 generally describes photographic elements employing high dye yield couplers having electrically neutral chromophores, and the contents

thereof are incorporated herein by reference. Further, particularly suitable couplers containing a methine dye chromophore are described in an application of Mooberry et al entitled "Photographic Element Containing A High Dye-Yield Coupler With A Methine Dye Chromophore" which is 5 cofiled herewith.

In one embodiment of the invention, when the ClogP is appropriately selected, it is believed that mobility of the —L-DYE or —(T)<sub>m</sub>—L-DYE fragment is permitted while the linking group is attached to the second dye but, once the linking group is cleaved from the second dye, diffusion of DYE is no longer possible. This result is achieved through the provision that the second dye has a calculated neutral 10 partition coefficient (ClogP) in the range of 3.5 to 5.5. Thus, when the linking group is cleaved from the second dye, the 15 dye no longer contains the charged highly polar portion represented by the linking group. It follows that the second dye is no longer free to diffuse after the linking group has separated and this provides good stability of the image dye 20 from the standpoint of long term image stability.

The neutral partition coefficient is the ratio of the distribution at equilibrium of a compound between octanol and water. The calculated values are derived using Medchem 25 software, version 3.54, Medical Chemistry Project, Pomona College, Claremont, California. For a recent discussion of this method see Albert J. Leo, in "Comprehensive Medicinal Chemistry", edited by C. Hansch, P. G. Sammes, and J. B. Taylor, Pergamon Press, New York, Volume 4, 1990).

The coupler of the invention releases a second dye having an electrically neutral chromophore. By this is meant that the chromophore at its characteristic hue bears no formal electrical charge. The second dye of the invention suitably contains a substituted nitrogen group which is bonded to the linking group. Such dyes may be any of the types disclosed, for example, in the aforementioned U.S. Pat. No. 4,840,884 and may be synthesized as described therein.

The DYE as described includes any releasable, electrically neutral dye that enables dye hue stabilization without mordanting the dye formed. The release mechanism can be initiated by oxidized reducing agent.

In U.S. Pat. No. 4,840,884, the term DYE is defined so that the adjacent nitrogen atom is not a part of DYE while 40 the definition herein does include the nitrogen atom. In either case, the composition of the dye formed by release is the same.

The R<sup>1</sup> substituent on —NR<sup>1</sup>— can be any substituent that does not adversely affect the coupler. When the —NR<sup>1</sup>— is part of an auxochrome, R<sup>1</sup> can be, for example, hydrogen or alkyl, such as alkyl containing 1 to 42 carbon atoms, including methyl, ethyl, propyl, n-butyl, t-butyl or eicosyl, or aryl, such as phenyl. When the nitrogen atom attached to L is part of a chromophore, R<sup>1</sup> becomes an integral part of the chromophore. Preferred R<sup>1</sup> groups are alkyl, such as alkyl containing 1 to 18 carbon atoms when R<sup>1</sup> is part of the dye auxochrome. R<sup>1</sup> when part of the chromophore is, for example, unsubstituted or substituted aryl, such as phenyl.

The selection of the type and size of the substituents of DYE can be made in order to provide a partition coefficient of DYE which permits the desired degree of diffusion.

Particularly useful classes of DYE moieties are:

I. Azo dye moieties including the —NR<sup>1</sup>— group represented by the structure:



wherein R<sup>25</sup> is hydrogen or a substituent, such as alkyl and R<sup>26</sup> and R<sup>27</sup> independently represent hydrogen or one or more substituents such as alkyl.

II. Azamethine dye moieties including the —NR<sup>1</sup>— group represented by the structure:



wherein R<sup>28</sup> is hydrogen or one or more substituents, such as alkyl; R<sup>29</sup> is hydrogen or a substituent, such as alkyl; and EWG is an electron withdrawing group.

III. Methine dye moieties including the —NR<sup>1</sup>— group represented by the structure:



wherein R<sup>30</sup> and R<sup>31</sup> are independently hydrogen or a substituent, such as alkyl; R<sup>30a</sup> is hydrogen or one or more substituents such as alkyl; and EWG is an electron withdrawing group having a positive Hammett's sigma(para) value.

The term DYE also includes dye precursors wherein the described substituted nitrogen atom is an integral part of the chromophore, also described herein as leuco dye moieties. Such dye precursors include, for example:



60 wherein R<sup>32</sup> is a group that is cleaved during processing to leave NH, or N=N, and R<sup>33</sup> is aryl, such as substituted phenyl.



wherein R<sup>34</sup> is a group that is cleaved during processing to leave NH, or N=C; and EWG is an electron withdrawing group as defined above.

Examples of cyan, magenta, yellow and leuco dyes are as follows:

A. Cyan



wherein R<sup>35</sup> is a substituent that does not adversely affect the dye, such as alkyl; R<sup>36</sup> is a substituent, such as an electron releasing group having a Hammett's sigma(para) value less than 0; and R<sup>37</sup> is one or more substituents, such as a strong electron withdrawing group having a Hammett's sigma (para) value of at least 0.23.

5



10

wherein R<sup>41</sup> is alkyl; R<sup>42</sup> is alkoxy, alkyl, or H; and R<sup>43</sup> is alkyl or H; and

20



25

30

wherein R<sup>44</sup> is alkyl; R<sup>45</sup> is alkoxy, alkyl, or H; R<sup>46</sup> is alkyl or aryl; and X is —O— or —NR\*— where R\* is H, alkyl, or aryl.

35

B. Magenta



wherein R<sup>38</sup> is a substituent that does not adversely affect the dye, such as alkyl; R<sup>39</sup> is a substituent, such as an electron releasing group as defined above; and R<sup>40</sup> is a substituent, such as a strong electron withdrawing group as defined above.

40



45

50

wherein R<sup>47</sup> and R<sup>48</sup> are individually hydrogen or alkyl; R<sup>49</sup> is an electron releasing group as defined above; and R<sup>51</sup> is a strong electron withdrawing group as defined above.



wherein R<sup>52</sup> and R<sup>54</sup> are individually hydrogen or a substituent; R<sup>53</sup> is —NHR<sup>a</sup> or —NHSO<sub>2</sub>R<sup>a</sup> wherein R<sup>a</sup> is a substituent; and R<sup>55</sup> and R<sup>56</sup> are individually hydrogen or a substituent.

The following are examples of suitable high dye yield 25  
couplers of the invention:



I-1



I-2



I-3

**11**

-continued



I-4



I-5



I-6

**12**

-continued



I-7



5

10

15

20

25

30

35

40

45

50

55

60

65



I-8

13

-continued



14

-continued



I-11



I-10



I-12

**15**

-continued

**16**

-continued

I-13

5



10

15

20

25

I-14

30

35

40

45

50

55

I-15

I-16



**17**

-continued



I-17

**18**

-continued



I-19

30

I-18



35

I-20



40

45

55

60

65

66

**19**

-continued



I-21

**20**

-continued



I-23



I-22



I-24

**21**

-continued

**22**

-continued



23

-continued



24

-continued



30



I-32



**25**

-continued



I-33

5

10

15

20

25

30



I-34

35

40

45

50

55

60

**26**

-continued

I-35



I-36

65

**27**

-continued



I-37

**28**

-continued



I-39



I-38



I-40



I-41



I-43

5

10

15

20

25

30

I-42

I-44



35

40

45

50

55

60



31

-continued



32

-continued

I-47



I-45

5

1

1

2

2

L-16

3

4

4

5

5

60

I-48



33

-continued



J-49

34

-continued



6

1

3

L-51

4

3

4

I-52



4

5

5

6

35

-continued



36

-continued

J-55



I-56



37

-continued



I-57

38

-continued



I-59

I-58

The chemical structure is a complex organic molecule with the following components from top to bottom:

- A carbonyl group ( $\text{C=O}$ ) attached to a tert-butyl group ( $\text{C}_2\text{H}_5$ ).
- A carbonyl group ( $\text{C=O}$ ) attached to an amide group ( $\text{NH-C(=O)-}$ ).
- An amide group ( $\text{NH-C(=O)-}$ ) attached to a 4-chlorophenyl group ( $\text{C}_6\text{H}_4\text{Cl}$ ).
- A carbonyl group ( $\text{C=O}$ ) attached to an oxygen atom ( $\text{O}$ ).
- An oxygen atom ( $\text{O}$ ) attached to a 4-aminophenylsulfonyl group ( $\text{NH-SO}_2\text{C}_6\text{H}_4\text{C}_6\text{H}_3\text{NH}_2$ ).
- A 4-aminophenylsulfonyl group ( $\text{NH-SO}_2\text{C}_6\text{H}_4\text{C}_6\text{H}_3\text{NH}_2$ ) attached to a 4-aminophenylsulfonyl group ( $\text{NH-SO}_2\text{C}_6\text{H}_4\text{C}_6\text{H}_3\text{NH}_2$ ).
- A carbonyl group ( $\text{C=O}$ ) attached to an oxygen atom ( $\text{O}$ ).
- An oxygen atom ( $\text{O}$ ) attached to a 4-(methylsulfonyl)butylamino group ( $\text{N}-(\text{CH}_2)_3\text{CH}_2\text{SO}_2\text{CH}_3$ ).
- A 4-(methylsulfonyl)butylamino group ( $\text{N}-(\text{CH}_2)_3\text{CH}_2\text{SO}_2\text{CH}_3$ ) attached to a 4-aminophenylsulfonyl group ( $\text{NH-SO}_2\text{C}_6\text{H}_4\text{C}_6\text{H}_3\text{NH}_2$ ).
- A carbonyl group ( $\text{C=O}$ ) attached to a 4-cyano-2-methylphenyl group ( $\text{C}_6\text{H}_3\text{CH}_2\text{C}_6\text{H}_3\text{CN}$ ).
- A 4-cyano-2-methylphenyl group ( $\text{C}_6\text{H}_3\text{CH}_2\text{C}_6\text{H}_3\text{CN}$ ) attached to an oxazoline ring ( $\text{N}=\text{C}(\text{CH}_3)=\text{O}$ ).
- An oxazoline ring ( $\text{N}=\text{C}(\text{CH}_3)=\text{O}$ ) attached to a 4-tert-butylphenyl group ( $\text{C}_6\text{H}_3\text{CH}_2\text{C}_6\text{H}_3\text{CH}_2\text{C}_2\text{H}_5$ ).



I-60

60

**39**

-continued

**40**

-continued



**41**

-continued

**42**

-continued

I-65



I-67

10

15

20

25

30

35

I-66

40

45

55

60

I-68

I-69



**43**

-continued



I-70



I-71



I-72

**44**

-continued



I-73



I-74



60



**45**

-continued



I-75

**46**

-continued



I-76 25



I-77



I-78

47

-continued



48

-continued



I-80



I-82



**49**

-continued

**50****50**

-continued

I-83

I-85



I-84

I-86



I-84



**51**

-continued



I-87

**52**

-continued

I-89



I-88



I-91



**53**

-continued



I-92

**54**

-continued



I-94

25

30

I-93



I-95



55

**55**

-continued



I-96

**56**

-continued



I-98



I-97



I-99



I-100

57

-continued



In addition to the foregoing, it may generally be desired that the photographic element of the invention contain reduced laydowns of silver and have a low molar ratio of dye theoretically formable from the coupler of the invention to silver present in the layer. More specifically, the element contains less than 90% of the silver typically employed in an

58

element employing conventional couplers and having the same sensitometry. It is not possible to specify the absolute levels of silver that may be employed since the amounts will vary depending on the coupler reactivities and many other components of the element. However, the applicable level of silver required for a conventional coupler to achieve a given aim sensitometry can be reduced significantly, i.e. by 10% to 35% and approaching 50% when the inventive couplers are used.

10 The present invention provides low silver laydowns in conjunction with low molar ratios of dye theoretically formable from the high dye yield couplers of the invention to silver. This enables not only conservation of the silver and dye required to attain the desired sensitometry, but also provides mass efficiency in the coupler necessary to produce 15 the necessary color image density and contrast.

It is possible to provide a coupler in accordance with the invention so that the first dye is ballasted to be completely immobile or so that it has limited mobility in the developer or other processing solution. It is also within the contemplation of the invention to include in association with the silver halide emulsion of the invention one or more additional couplers that are conventional image couplers or that are PUG releasing couplers, as described more fully herein.

The dyes formed by the coupler of the invention may be 25 within any desired color range. Yellow, cyan and magenta are the ranges most commonly used in color negative today. The first and second dyes of the invention are the same color if they have maximum absorbance in the same range, i.e. 400–500 nm, 500–600 nm, or 600–700 nm. Where the two 30 dyes are the same color they will typically have absorption maxima within 25 nm of each other. Photographic elements which may use the invention include image capture color negative, color print, and reversal to name a few.

negativ, color print, and reversal to name a few.

35 In a particularly suitable form of the invention, the silver halide layer of the invention represents at least one layer, preferably the fast or high sensitivity layer, of a multilayered color record. Such a layer is normally above the slower layers of the color record and contains a larger silver halide grain size for speed purposes. Use of the invention with  
40 respect to that layer provides significant improvement in granularity while permitting thinning of the layer allowing less degradation of the light image formed in underlying layers. The invention has particular suitability with tabular grains to enable superior grain reduction. It may also be  
45 desirable to employ the coupler of the invention in a slow imaging layer where finer grain emulsions are typically employed.

The desired results are enabled in part through providing low laydown of the imaging coupler and formable image 50 dye relative to the laydown of silver in the layer. Thus the molar ratio of formable dye (theoretical amount of first and second dye) to silver halide is less than 1.0. More suitably, the ratio is less than 0.8 and often less than 0.55 provides good results.

55 The developability of an emulsion refers to the ability of the emulsion to produce maximum density within the desired processing time. The Kodak C-41 process for color negative processing is described in The British Journal of Photography Annual of 1988, pp 191-98, provides for a 3.25  
60 minute development step. A slow developing emulsion will not be fully developed in the normal development time. It will continue to develop if the development time is extended. The developability of an emulsion is a function of many factors such as grain type, chemical sensitization,  
65 halide content etc.

For example, developability of an emulsion can be varied by changing the content of the particular halide(s) employed

in the emulsion. Developability may be lowered, for example, by increasing the iodide content, varying the iodide distribution, changing the grain size, changing the grain morphology, and by the degree of finishing in which the type or level of sensitization and additives which decrease fog formation are varied in the preparation of the emulsion.

Generally any known emulsions are useful in the invention including cubic three-dimensional type emulsions and tabular grain emulsions, all as described in the Research Disclosure publications cited herein. The emulsions may be poly- or monodisperse. In particular, emulsions containing at least 3 mol % iodide and typically at least 6 mol % iodide are suitable.

To be more specific, for the purposes of this description, an emulsion has "low developability" if coatings of it, compared to those of a standard emulsion (both coated with a conventional image coupler containing conventional image coupler C-1) having the same size, speed, and morphology, and capable of full development within the standard 3.25 minutes development time, the emulsion in question has for the same development time:

(a) a lower  $D_{min}$ , and

(b) a contrast of 90% or less,

both compared to the standard.

The C-41 process is described in The British Journal of Photography Annual of 1988, pages 191-198, as follows:

C-41 Procedure (after Kodak)

|                      |               |                     |
|----------------------|---------------|---------------------|
| 1 Colour development | 3 min/15 sec  | 37.8 $\pm$ 0.15° C. |
| 2 Bleach             | 4 min/20 sec  | 24-40° C.           |
| 3 Wash               | 1 min/05 sec  | 24-40° C.           |
| 4 Fix                | 4 min/20 sec  | 24-40° C.           |
| 5 Wash               | 3 min/15 sec  | 24-40° C.           |
| 6 Stabilization      | 1 min/05 sec  | 24-40° C.           |
| 7 Dry                | —             | <43° C.             |
| Total                | 17 min/20 sec |                     |

Operational Steps:

1. Prepare a water bath at 41° C.; this provides a thermal reservoir.
2. Bring the solutions up to 38° C. before use.
3. Fill the developing tank with the necessary quantity of developer, agitate continuously for 20 sec, then plunge it in the water bath to within 2-3 cm of the top of the lid.
4. Take the tank out again and agitate—preferably by inversion—for 5 sec. Put it back in the water bath. Repeat this cycle giving 6 agitations each minute.
5. Empty the tank 10 sec before the elapse of the require time. Shake it well so that as little colour developer as possible is left inside.
6. Pour in the bleach and carry out the same agitation rhythm as above.
7. When the bleach stage is finished, the tank may be opened to simplify washing.
8. Once it has come out of the stabilizing bath, the film is hung up to dry in the usual manner. In a normally heated and ventilated room it will be dry in about 30-40 min.

Formulae:

The quantities are given in grams per litre. The chemicals are dissolved in the indicated order.

Colour Developer (pH: 10.0-10.1)

|   |                                 |           |
|---|---------------------------------|-----------|
| 5 | Calgon                          | 2.0 g     |
|   | Sodium sulphite (anhydrous)     | 4.25 g    |
|   | Potassium bromide               | 1.5 g     |
|   | Potassium carbonate (anhydrous) | 37.5 g    |
|   | Hydroxylamine sulphate          | 2.0 g     |
|   | Water to make                   | 1000.0 ml |

Add 6 hr before use:

|    |                                                                                                                                        |         |
|----|----------------------------------------------------------------------------------------------------------------------------------------|---------|
| 10 | CD 4-4-[N-Ethyl-N-2-hydroxyethyl]-2-methylenephene-diamine sulphate = Colour Developer 4 (Merck), CD-4 (Kodak), or CD-4 (20% solution) | 4.75 g  |
| 15 | CD-4 stock solution                                                                                                                    | 24.0 ml |

The following keeps well for about 2 months in the cool away from light.

|    |                                        |           |
|----|----------------------------------------|-----------|
| 20 | CD-4                                   | 20.0 g    |
|    | Potassium metabisulphite (crystalline) | 3.0 g     |
|    | Water to make                          | 1000.0 ml |

Bleach:

|    |                   |           |
|----|-------------------|-----------|
| 25 | EDTA NaFe         | 100.0 g   |
|    | Potassium bromide | 50.0 g    |
|    | Ammonia 20%       | 6.0 ml    |
|    | Water to make     | 1000.0 ml |

Fix (pH: 5.8-6.5)

|    |                                        |           |
|----|----------------------------------------|-----------|
| 30 | Ammoniumthiosulphite                   | 120.0 g   |
|    | Sodium sulphite (anhydrous)            | 20.0 g    |
|    | Potassium metabisulphite (crystalline) | 20.0 g    |
|    | Water to make                          | 1000.0 ml |
|    | Stabilizer                             |           |
|    | Wetting agent (10% solution)           | 10.0 ml   |

35 The method of the invention provides for the exposure of a photographic element of the invention followed by contacting the element with a color developing chemical to form a color image. Color forming chemicals are described more fully hereinafter.

40 As used herein, the term substituent, unless otherwise specifically stated, has a broad definition. The substituent may be, for example, halogen, such as chlorine, bromine or fluorine; nitro; hydroxyl; cyano; and  $-\text{CO}_2\text{H}$  and its salts; and groups which may be further substituted, such as alkyl, including straight or branched chain alkyl, such as methyl, trifluoromethyl, ethyl, t-butyl, 3-(2,4-di-t-amylphenoxy)propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, 50 tetradecyloxy 2-(2,4-di-t-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetrade canamido, alpha-(2,4-di-t-pentylphenoxy)acetamido, alpha-(2,4-di-t-pentylphenoxy)butyramido, alpha-(3-pentadecylphenoxy)hexanamido, alpha-(4-hydroxy-3-t-butylphenoxy)tetradecanamido, 2-oxo-pyrrolidin-1-yl, 2-oxo-5-tetradecylpyrrolin-1-yl, 60 N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzoyloxycarbonylamino, hexadecyloxycarbonylamino, 65 2,4-di-t-butylphenoxy carbonylamino, phenyl carbonylamino, 2,5-(di-t-pentylphenyl) carbonylamino, p-dodecylphenyl carbonylamino,

p-tolylcarbonylamino, N-methylureido, N,N-dimethylureido, N-methyl-N-dodecylureido, N-hexadecylureido, N,N-dioctadecylureido, N,N-diethyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as methylsulfonamido, benzenesulfonamido, p-tolylsulfonamido, p-dodecylbenzenesulfonamido, N-methyltetradecylsulfonamido, N,N-dipropylsulfamoylamino, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecylxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; acyl, such as acetyl, (2,4-di-t-aminophenoxy)acetyl, phenoxy carbonyl, p-dodecylphenoxy carbonyl methoxycarbonyl, butoxycarbonyl, tetradecyloxycarbonyl, ethoxycarbonyl, benzyloxycarbonyl, 3-pentadecyloxycarbonyl, and dodecylloxycarbonyl; sulfonyl, such as methoxysulfonyl, octyloxysulfonyl, tetradecyloxysulfonyl, 2-ethylhexyloxysulfonyl, phenoxy sulfonyl, 2,4-di-t-pentylphenoxy sulfonyl, methylsulfonyl, octylsulfonyl, 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy)ethylthio, phenylthio, 2-butoxy-5-t-octylphenylthio, and p-tolylthio; acyloxy, such as acetoxy, benzyloxy, octadecanoxy, p-dodecylamido benzoyloxy, N-phenylcarbamoyloxy, N-ethylcarbamoyloxy, and cyclohexylcarbamoyloxy; amine, such as phenylanilino, 2-chloroanilino, diethylamine, dodecylamine; imino, such as 1 (N-phenylimido)ethyl, N-succinimido or 3-benzylhydantoinyl; phosphate, such as dimethylphosphate and ethylbutylphosphate; phosphite, such as diethyl and dihexylphosphite; azo, such as phenylazo and naphthylazo; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyloxy; quaternary ammonium, such as triethylammonium; and silyloxy, such as trimethylsilyloxy.

The particular substituents used may be selected to attain the desired photographic properties for a specific application and can include, for example, hydrophobic groups, solubilizing groups, blocking groups, etc. Generally, the above groups and substituents thereof may typically include those having 1 to 42 carbon atoms and usually less than 24 carbon atoms, but greater numbers are possible depending on the particular substituents selected. Moreover, as indicated, the substituents may themselves be suitably substituted with any of the above groups.

The materials of the invention can be used in any of the ways and in any of the combinations known in the art. Typically, the invention materials are combined with a silver

halide emulsion and the mixture is coated as a layer on a support to form part of a photographic element. Alternatively, they can be incorporated at a location adjacent to the silver halide emulsion layer where, during development, they will be in reactive association with development products such as oxidized color developing agent. Thus, as used herein, the term "associated" signifies that the compound is in the silver halide emulsion layer or in an adjacent location where, during processing, it is capable of reacting with silver halide development products.

It may be desirable to include a high molecular weight hydrophobe or "ballast" group in the component molecule to control the migration of various components. Representative ballast groups include substituted or unsubstituted alkyl or aryl groups containing 8 to 42 carbon atoms. Representative substituents on such groups include alkyl, aryl, alkoxy, aryloxy, alkylthio, hydroxy, halogen, alkoxy carbonyl, aryloxy carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers, subbing layers, and the like.

If desired, the photographic element can be used in conjunction with an applied magnetic layer as described in *Research Disclosure*, November 1992, Item 34390 published by Kenneth Mason Publications, Ltd. Dudley Annex, 12a North Street, Emsworth, Hampshire P010 7DQ, ENGLAND; and in U.S. Pat. Nos. 5,252,441; 5,254,449; and 5,254,446; the contents of which are incorporated herein by reference.

Color negative films employing such layers can be employed, in combination with cameras that can record and cause to be stored on such a layer, various useful information related to the use and history of the film. Specific examples include exposure information on a per scene and per roll basis. These films can then be processed in automated processing apparatus that can retrieve film characteristic information as well as film exposure and use information, and optionally modify the processing to ensure optimal performance and optionally record the details of processing of the magnetic layer. The films can then be printed using automated printers that can retrieve both film and process history information and optionally alter, based on the information, exposure characteristics chosen from printing

time, printing light intensity, printing light color balance, printing light color temperature, printing magnification or printing lens adjustment, exposure, or printing time, and the color filters so as to enable production of well-balanced display prints from various color originating materials. These layers can be located on the same side of the support as light sensitive layers or arranged so that the support is between the magnetic layer and the light sensitive layers. This information is useful in altering film processing and printing conditions so as to aid in producing a pleasing image.

It is specifically contemplated to employ supports bearing magnetic layers as described.

In the following discussion of suitable materials for use in the emulsions and elements of this invention, reference will be made to *Research Disclosure*, December 1989, Item 308119, available as described above, which will be identified hereafter by the term "Research Disclosure." The contents of the Research Disclosure, including the patents and publications referenced therein, are incorporated herein by reference, and the Sections hereafter referred to are Sections of the Research Disclosure. The materials of the invention may also be used in conjunction with the materials described in *Koukai Gihou No. 94-6023*, Hatsumei Kyoushikai, March 1994, available from the Japanese Patent Office, which is incorporated herein by reference.

The silver halide emulsions employed in the elements of this invention can be either negative-working or positive-working. Suitable emulsions and their preparation as well as methods of chemical and spectral sensitization are described in Sections I through IV. Color materials and development modifiers are described in Sections VII and XXI. Vehicles are described in Section IX, and various additives such as brighteners, antifoggants, stabilizers, light absorbing and scattering materials, hardeners, coating aids, plasticizers, lubricants and matting agents are described, for example, in Sections V, VI, VIII, X, XI, XII, and XVI. Manufacturing methods are described in Sections XIV and XV, other layers and supports in Sections XIII and XVII, processing methods and agents in Sections XIX and XX, and exposure alternatives in Section XVIII.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction and the like.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocycl, sulfonamido, mercaptotetrazole, benzothiazole, mercaptopropionic acid, phosphonyloxy, arylthio, and arylazo. These coupling-off groups are described in the art, for example, in U.S. Pat. Nos. 2,455, 169, 3,227,551, 3,432,521, 3,476,563, 3,617,291, 3,880,661, 4,052,212 and 4,134,766; and in U.K. Patents and published application Nos. 1,466,728, 1,531,927, 1,533,039, 2,006, 755A and 2,017,704A, the disclosures of which are incorporated herein by reference.

It may be useful to use a combination of couplers any of which may contain known ballasts or coupling-off groups

such as those described in U.S. Pat. Nos. 4,301,235; 4,853, 319 and 4,351,897. The coupler may contain solubilizing groups such as described in U.S. Pat. No. 4,482,629. The coupler may also be used in association with "wrong" colored couplers (e.g. to adjust levels of interlayer correction) and, in color negative applications, with masking couplers such as those described in EP 213,490; Japanese Published Application 58-172,647; U.S. Pat. Nos. 2,983, 608; 4,070,191; and 4,273,861; German Applications DE 2,706,117 and DE 2,643,965; U.K. Patent 1,530,272; and Japanese Application A-113935. The masking couplers may be shifted or blocked, if desired.

For example, in a color negative element, the materials of the invention may replace or supplement the materials of an element comprising a support bearing the following layers from top to bottom:

- (1) one or more overcoat layers containing ultraviolet absorber(s);
- (2) a two-coat yellow pack with a fast yellow layer containing "Coupler 1": Benzoic acid, 4-chloro-3-((2-(4-ethoxy-2,5-dioxo-3-(phenylmethyl)-1-imidazolidinyl)-3-(4-methoxyphenyl)-1,3-dioxopropyl)amino)—, dodecyl ester and a slow yellow layer containing the same compound together with "Coupler 2": Propanoic acid, 2-[[5-[[4-[2-[[2,4-bis(1,1-dimethylpropyl)phenoxy]acetyl]amino]-5-[2,2,3,3,4,4,4-4-heptafluoro-1-oxobutyl]amino]-4-hydroxyphenoxy]-2,3-dihydroxy-6-[(propylamino)carbonyl]phenyl]thio]-1,3,4-thiadiazol-2-yl]thio]-, methyl ester and "Coupler 3": 1-((dodecyloxy)carbonyl) ethyl(3-chloro-4-((3-(2-chloro-4-((1-tridecanoylethoxy) carbonyl)anilino)-3-oxo-2-((4)(5)(6)-(phenoxy carbonyl)-1H-benzotriazol-1-yl)propanoyl)amino))benzoate;
- (3) an interlayer containing fine metallic silver;
- (4) a triple-coat magenta pack with a fast magenta layer containing "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)—, "Coupler 5": Benzamide, 3-((2-(2,4-bis(1,1-dimethylpropyl)phenoxy)-1-oxobutyl)amino)-N-(4',5'-dihydro-5'-oxo-1'-(2,4,6-trichlorophenyl)(1,4'-bi-1H-pyrazol)-3'-yl)—, "Coupler 6": Carbamic acid, (6-(((3-(dodecyloxy)propyl) amino)carbonyl)-5-hydroxy-1-naphthalenyl)—, 2-methylpropyl ester, "Coupler 7": Acetic acid, ((2-((3-((3-(dodecyloxy)propyl)amino)carbonyl)-4-hydroxy-8-(((2-methylpropoxy)carbonyl) amino)-1-naphthalenyl)oxy)ethyl)thio)—, and "Coupler 8": Benzamide, 3-((2-(2,4-bis(1,1-dimethylpropyl)phenoxy)-1-oxobutyl)amino)-N-(4,5-dihydro-4-((4-methoxyphenyl) azo)-5-oxo-1-(2,4,6-trichlorophenyl)-1H-pyrazol-3-yl); a mid-magenta layer and a slow magenta layer each containing "Coupler 9": a ternary copolymer containing by weight in the ratio 1:1:2 2-Propenoic acid butyl ester, styrene, and N-[1-(2,4,6-trichlorophenyl)-4,5-dihydro-5-oxo-1H-pyrazol-3-yl]-2-methyl-2-propenamide; and "Coupler 10": Tetradecanamide, N-(4-chloro-3-((4-((2,2-dimethyl-1-oxopropyl)amino)phenyl)azo)-4,5-dihydro-5-oxo-1-(2,4,6-trichlorophenyl)-1H-pyrazol-3-yl)amino)phenyl)—, in addition to Couplers 3 and 8;
- (5) an interlayer;
- (6) a triple-coat cyan pack with a fast cyan layer containing Couplers 6 and 7; a mid-cyan containing Coupler 6 and "Coupler 11": 2,7-Naphthalenedisulfonic acid,

**65**

5-(acetylamino)-3-((4-(2-((3-((3-(2,4-bis(1,1-dimethylpropyl)phenoxy) propyl)amino)carbonyl)-4-hydroxy-1-naphthalenyl) oxy)ethoxy)phenyl)azo)-4-hydroxy—, disodium salt; and a slow cyan layer containing Couplers 2 and 6;

5

- (7) an undercoat layer containing Coupler 8; and
- (8) an antihalation layer.

In a color paper format, the materials of the invention may replace or supplement the materials of an element comprising a support bearing the following layers from top to bottom:

- (1) one or more overcoats;
- (2) a cyan layer containing “Coupler 1”: Butanamide, 2-(2,4-bis(1,1-dimethylpropyl)phenoxy)-N-(3,5-dichloro-2-hydroxy-4-methylphenyl)—, “Coupler 2”: Acetamide, 2-(2,4-bis(1,1-dimethylpropyl)phenoxy)-N-(3,5-dichloro-2-hydroxy-4—, and UV Stabilizers: Phenol, 2-(5-chloro-2H-benzotriazol-2-yl)-4,6-bis(1,1-dimethylethyl)—; Phenol, 2-(2H-benzotriazol-2-yl)-4-(1,1-dimethylethyl)-6-(1-methylpropyl)—; and Phenol, 2-(2H-benzotriazol-2-yl)-4,6-bis(1,1-dimethylpropyl)— and a poly(t-butylacrylamide) dye stabilizer;
- (3) an interlayer;
- (4) a magenta layer containing “Coupler 3”: Octanamide, 2-[2,4-bis(1,1-dimethylpropyl)phenoxy]-N-[2-(7-chloro-6-methyl-1H-pyrazolo[1,5-b][1,2,4]triazol-2-yl)propyl]— together with 1,1'-Spirobi(1H-indene), 2,2',3,3'-tetrahydro-3,3,3',3'-tetramethyl-5,5',6,6'-tetrapropoxy—;
- (5) an interlayer; and
- (6) a yellow layer containing “Coupler 4”: 1-Imidazolidineacetamide, N-(5-((2-(2,4-bis(1,1-dimethylpropyl)phenoxy)-1-oxobutyl)amino)-2-chlorophenyl)-alpha-,(2,2-dimethyl-1-oxopropyl)-4-ethoxy-2,5-dioxo-3-(phenylmethyl)—.

In a reversal format, the materials of the invention may replace or supplement the materials of an element comprising a support bearing the following layers from top to bottom:

- (1) one or more overcoat layers;
- (2) a nonsensitized silver halide containing layer;
- (3) a triple-coat yellow layer pack with a fast yellow layer containing “Coupler 1”: Benzoic acid, 4-(1-((2-chloro-5-((dodecylsulfonyl)amino)phenyl) amino)carbonyl)-3,3-dimethyl-2-oxobutoxy)—, 1-methylethyl ester; a mid yellow layer containing Coupler 1 and “Coupler 2”: Benzoic acid, 4-chloro-3-[[2-[4-ethoxy-2,5-dioxo-3-(phenylmethyl)-1-imidazolidinyl]-4,4-dimethyl-1,3-dioxopentyl] amino]—, dodecylester; and a slow yellow layer also containing Coupler 2;
- (4) an interlayer;
- (5) a layer of fine-grained silver;
- (6) an interlayer;
- (7) a triple-coated magenta pack with a fast and mid magenta layer containing “Coupler 3”: 2-Propenoic acid, butyl ester, polymer with N-[1-(2,5-dichlorophenyl)-4,5-dihydro-5-oxo-1H-pyrazol-3-yl]-2-methyl-2-propenamide; “Coupler 4”: Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-; and “Coupler 5”:

**66**

Benzamide, 3-((2,4-bis(1,1-dimethylpropyl)phenoxy) acetyl)amino)-N-(4,5-dihydro-5-oxo-1-(2,4,6-trichlorophenyl)-1H-pyrazol-3-yl)—; and containing the stabilizer 1,1'-Spirobi(1H-indene), 2,2',3,3'-tetrahydro-3,3,3',3'-tetramethyl-5,5',6,6'-tetrapropoxy-; and in the slow magenta layer Couplers 4 and 5 with the same stabilizer;

- (8) one or more interlayers possibly including fine-grained nonsensitized silver halide;
- (9) a triple-coated cyan pack with a fast cyan layer containing “Coupler 6”: Tetradecanamide, 2-(2-cyanophenoxy)-N-(4-((2,2,3,3,4,4,4-heptafluoro-1-oxobutyl)amino)-3-hydroxyphenyl)—; a mid cyan containing “Coupler 7”: Butanamide, N-(4-((2-(2,4-bis(1,1-dimethylpropyl)phenoxy)-1-oxobutyl)amino)-2-hydroxyphenyl)-2,2,3,3,4,4,4-heptafluoro— and “Coupler 8”: Hexanamide, 2-(2,4-bis(1,1-dimethylpropyl)phenoxy)-N-(4-((2,2,3,3,4,4,4-heptafluoro-1-oxobutyl)amino)-3-hydroxyphenyl)—; and a slow cyan layer containing Couplers 6, 7, and 8;
- (10) one or more interlayers possibly including fine-grained nonsensitized silver halide; and
- (11) an antihalation layer.

The inventive materials may be used in association with materials that accelerate or otherwise modify the processing steps e.g. of bleaching or fixing to improve the quality of the image. Bleach accelerator releasing couplers such as those described in EP 193,389; EP 301,477; U.S. Pat. Nos. 4,163,669; 4,865,956; and 4,923,784, may be useful. Also contemplated is use of the compositions in association with nucleating agents, development accelerators or their precursors (UK Patent 2,097,140; U.K. Patent 2,131,188); electron transfer agents (U.S. Pat. Nos. 4,859,578; 4,912,025); anti-fogging and anti color-mixing agents such as derivatives of hydroquinones, aminophenols, amines, gallic acid; catechol; ascorbic acid; hydrazides; sulfonamidophenols; and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with “smearing” couplers (e.g. as described in U.S. Pat. No. 4,366,237; EP 96,570; U.S. Pat. Nos. 4,420,556; and 4,543,323.) Also, the compositions may be blocked or coated in protected form as described, for example, in Japanese Application 61/258,249 or U.S. Pat. No. 5,019,492.

The invention materials may further be used in combination with image-modifying compounds such as “Developer Inhibitor-Releasing” compounds (DIR’s). DIR’s useful in conjunction with the compositions of the invention are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography," C. R. Barr, J. R. Thirtle and P. W. Vittum in *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, <sup>15</sup> selenobenzothiazoles, mercaptobenzoxazoles, selenobenzoxazoles, mercaptobenzimidazoles, selenobenzimidazoles, benzodiazoles, mercaptooxazoles, mercaptotriazoles, mercaptooxadiazoles, mercaptodiazoles, mercaptooxathiazoles, tellurotetrazoles or benzisodiazoles. In a preferred embodiment, the inhibitor moiety or group is selected from the following formulas:



wherein  $R_I$  is selected from the group consisting of straight and branched alkyls of from 1 to about 8 carbon atoms, benzyl, phenyl, and alkoxy groups and such groups containing none, one or more than one such substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group consisting of hydrogen, halogens and alkoxy, phenyl and carbonamido groups,  $-COOR_V$  and  $-NHOOR_V$  wherein  $R_V$  is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers).

As mentioned, the developer inhibitor-releasing coupler may include a timing group, which groups have been described earlier with respect to the high dye-yield coupler of the invention. Suitable developer inhibitor-releasing couplers for use in the present invention include, but are not limited to, the following:

D1



69

-continued

70

D2



D3



D4



D5







It is also contemplated that the concepts of the present invention may be employed to obtain reflection color prints as described in *Research Disclosure*, November 1979, Item 18716, available from Kenneth Mason Publications, Ltd, Dudley Annex, 12a North Street, Emsworth, Hampshire PO101 7DQ, England, incorporated herein by reference. Materials of the invention may be coated on pH adjusted support as described in U.S. Pat. No. 4,917,994; on a support with reduced oxygen permeability (EP 553,339); with epoxy solvents (EP 164,961); with nickel complex stabilizers (U.S. Pat. Nos. 4,346,165; 4,540,653 and 4,906,559 for example); with ballasted chelating agents such as those in U.S. Pat. No. 4,994,359 to reduce sensitivity to polyvalent cations such as calcium; and with stain reducing compounds such as described in U.S. Pat. No. 5,068,171. Other compounds useful in combination with the invention are disclosed in Japanese Published Applications described in Derwent Abstracts having accession numbers as follows: 90-072,629, 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

Especially useful in this invention are tabular grain silver halide emulsions. Specifically contemplated tabular grain emulsions are those in which greater than 50 percent of the total projected area of the emulsion grains are accounted for by tabular grains having a thickness of less than 0.3 micron (0.5 micron for blue sensitive emulsion) and an average tabularity (T) of greater than 25 (preferably greater than 100), where the term "tabularity" is employed in its art recognized usage as

$$T = ECD/t^2$$

where

ECD is the average equivalent circular diameter of the tabular grains in micrometers and  
t is the average thickness in micrometers of the tabular grains.

The average useful ECD of photographic emulsions can range up to about 10 micrometers, although in practice emulsion ECD's seldom exceed about 4 micrometers. Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim

tabular grain projected areas be satisfied by thin ( $t < 0.2$  micrometer) tabular grains. To achieve the lowest levels of granularity it is preferred that aim tabular grain projected areas be satisfied with ultrathin ( $t < 0.06$  micrometer) tabular grains. Tabular grain thicknesses typically range down to about 0.02 micrometer. However, still lower tabular grain thicknesses are contemplated. For example, Daubendiek et al U.S. Pat. No. 4,672,027 reports a 3 mole percent iodide tabular grain silver bromoiodide emulsion having a grain thickness of 0.017 micrometer. Ultrathin tabular grain high chloride emulsions are disclosed by Maskasky U.S. Pat. No. 5,217,858.

As noted above tabular grains of less than the specified thickness account for at least 50 percent of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabular grains satisfying the thickness criteria above account for at least 90 percent of total grain projected area.

Suitable tabular grain emulsions can be selected from among a variety of conventional teachings, such as those of the following: Research Disclosure, Item 22534, January 1983, published by Kenneth Mason Publications, Ltd., Emsworth, Hampshire PO10 7DD, England; U.S. Pat. Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069 and 5,061,616.

Silver chloride tabular grains useful in this invention include those having {100} major faces. These grains are both morphologically stable and capable of being readily sensitized with a variety of sensitizing dyes. Silver chloride emulsions characterized by at least 50 percent of the grain population projected area being accounted for by tabular grains (1) bounded by {100} major faces having adjacent edge ratios of less than 10 and (2) each having an aspect ratio of at least 2, as described by House et al in allowed U.S. application Ser. No. 112,489 and by Maskasky in U.S. Pat. No. 5,264,337 and allowed U.S. Ser. No. 035,349 the disclosures of which are incorporated herein by reference, are suitable for the invention.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive

emulsions of the unfogged, internal latent image-forming type, which are positive-working when development is conducted with uniform light exposure or in the presence of a nucleating agent.

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye.

With negative-working silver halide, the processing step described above provides a negative image. The described elements can be processed in the known C-41 color process as described in The British Journal of Photography Annual of 1988, pages 191-198. Where applicable, the element may be processed in accordance with color print processes such as the RA-4 process of Eastman Kodak Company as described in the British Journal of Photography Annual of 1988, Pp 198-199. To provide a positive (or reversal) image, the color development step can be preceded by development with a non-chromogenic developing agent to develop exposed silver halide, but not form dye, and followed by uniformly fogging the element to render unexposed silver halide developable. Alternatively, a direct positive emulsion can be employed to obtain a positive image.

Preferred color developing agents are p-phenylenediamines such as:

4-amino-N,N-diethylaniline hydrochloride,  
4-amino-3-methyl-N,N-diethylaniline hydrochloride,  
4-amino-3-methyl-N-ethyl-N-( $\beta$ -(methanesulfonamido)ethyl) aniline sesquisulfate hydrate,  
4-amino-3-methyl-N-ethyl-N-( $\beta$ -hydroxyethyl)aniline sulfate,  
4-amino-3- $\beta$ -(methanesulfonamido)ethyl-N,N-diethylaniline hydrochloride and  
4-amino-N-ethyl-N-(2-methoxyethyl)-m-toluidine di-p-toluene sulfonic acid.

Development is usually followed by the conventional steps of bleaching, fixing, or bleach-fixing, to remove silver or silver halide, washing, and drying.

It is understood throughout this specification and claims that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form, but also its form further substituted with any photographically useful substituents. Usually the further substituent will have less than 30 carbon atoms and typically less than 20 carbon atoms.

The couplers of the invention can be prepared by methods known in the organic synthesis art including those methods described in U.S. Pat. No. 4,840,884.

## Coupler Synthesis

Preparation of Coupler Having the Formula:



The overall scheme for the synthesis of the coupler is illustrated in Scheme I. The linking group intermediate 10 was prepared in four steps. Commercially available methyl-p-amino benzoate (78.6 g, 0.52 mole) was dissolved in about 500 mL of methylene chloride containing 2,6-lutidine (56 g, 0.52 mole, 60.7 mL), cooled in an ice bath, and treated with trifluoromethane sulfonic anhydride (146 g, 0.52 mole/l in 50 mL of methylene chloride) dropwise over 5 min. The reaction mixture was warmed to room temperature over 30 min before washing with excess 2N HCl. The organic phase was then washed four times with 250 mL portions of 1N NaHCO<sub>3</sub>. The aqueous washes were acidified with 12N HCl to precipitate a creamy solid which was collected, washed with water, and air dried to yield 86 g of the trifluoromethylsulfonamide (methyl-p-trifluoromethyl-sulfonamido benzoate). This trifluoromethylsulfonamide (86 g, 0.3 mole) was added to a stirred solution of NaOH (55 g, 1.38 mole) in 660 mL of water. The mixture was stirred for about 15 min before acidifying with excess 2N HCl to yield a precipitate that was collected, washed with water, and air dried to yield 72 g of the saponified benzoic acid. This benzoic acid (74.9 g, 0.278 mole) was converted to acid chloride by stirring in a mixture of 350 mL ethyl acetate, 3 drops of DMF, and 53 g (0.417 mole) oxalyl chloride for 3 hr. Solvents were distilled off under vacuum and residual oxalyl chloride was chased three times with a mixture of 150 mL methylene chloride and 50 mL heptane. The crude oil was mixed with 25 mL of heptane and placed in a refrigerator overnight. The crystals that formed were slurried in about 200 mL of heptane and air dried to yield 57.6 g of the acid chloride. This acid chloride (57.6 g, 0.198 mole, in 100 mL tetrahydrofuran) was added dropwise over 10 min with good stirring to a solution of 3-amino-4-hydroxy benzyl alcohol (27.5 g, 0.198 mole) in 100 mL of pyridine cooled to 5° C.

in a 3-neck round-bottomed flask fitted with mechanical stirrer. After 30 min at room temperature, the reaction mixture was diluted with 300 mL of ethyl acetate and washed with excess 2N HCl and water. The organic layer 5 was dried over MgSO<sub>4</sub> and stripped to a crude oil that crystallized rapidly with addition of 200 mL heptane. The crystals were collected and air dried to yield 69 g of the linking group 10. This linking group 10 was attached to coupler 11 by combining 32 g (0.082 mole) of 10 and 48.5 10 g (0.082 mole) of 11 with 200 mL of DMF and treating with tetramethylguanidine (18.8 g, 0.164 mole). The reaction mixture was stirred for 2 hr and then diluted with ethyl acetate and washed with excess 1N HCl and water. The organic layer was dried over MgSO<sub>4</sub> and concentrated to an 15 oil. The oil was dissolved in 2 parts of ethyl acetate and diluted with 8 parts heptane. The solvents were evaporated with stirring to yield brown crystals. These crystals were slurried in heptane, collected, and air dried to yield about 60 g of coupler the target coupler.

20 The dye intermediate 13 was prepared according to Scheme II, illustrated below. Commercially available 2,5-dimethylaniline (50 g, 0.413 mole) was added to formic acid (46 g, 1 mole, 38 mL) in a round-bottomed flask fitted with a condenser and heating mantle. The mixture was heated to 25 reflux for 2 hr and then cooled to room temperature before pouring into 2 L of cold water with good stirring. The resulting precipitate was collected and air dried to yield 61 g of the formamide (2,5-dimethylformanilide). This formamide (59.6 g, 0.4 mole) and bromodecane (104.6 g, 0.4 30 mole) were mixed with 40 mL t-butanol and 400 mL THF in a 3-neck round-bottomed flask fitted with a reflux condenser, heating mantle, and nitrogen purge. The mixture was treated with potassium t-butoxide (49.2 g), heated to reflux for 12 hr, cooled to room temperature, and diluted 35 with ethyl acetate. The mixture was then washed with excess 1N HCl and water. The organic layer was dried over MgSO<sub>4</sub> and concentrated to yield about 120 g of crude alkylated formamide. Alkylated formamide (120 g, 0.38 mole) was dissolved in 420 mL acetic acid and 120 mL 12N HCl and 40 heated to reflux for 16 hr. The solvents were distilled off under vacuum, and the resulting solid was collected and air dried to yield 107 g of the corresponding amine hydrochloride (2,5-dimethyl-N-dodecyl aniline hydrochloride). This amine hydrochloride (34.2 g, 0.105 mole) was mixed with 250 mL acetic acid, 20 mL 12N HCl, and 20 mL formaldehyde in a large mouth 3-L round-bottomed flask fitted with a mechanical stirrer and a heating mantle. The mixture was heated to about 80° C. before removing the heat and 45 treating with N,N-dimethylnitrosoaniline (22.5 g, 0.15 mole) in portions over a 10-min interval with good stirring. The solvents were distilled off under vacuum and the resulting oil was dissolved in 300 mL of ethyl acetate and excess 2N HCl. The aqueous phase was washed an additional three 50 times with 300 mL portions of ethyl acetate. These ethyl acetate extracts were passed through a pad of silica gel before removing solvent under vacuum to yield a slurry that crystallized with the addition of 500 mL of heptane. The crystals were collected and air dried to yield 17 g of the aldehyde (2,5-dimethyl-4-dodecylamino-benzaldehyde; 55 DMBA).

Commercially available 4-t-butyl phenol (30 g, 0.2 mole) was dissolved in 200 mL ethyl acetate in a 600-mL round-bottomed flask fitted with a mechanical stirrer, and cooled to 0° C. The mixture was treated with nitric acid (13 mL, in 13 mL water) dropwise over 10 min and then a catalytic amount of NaNO<sub>2</sub>. After 45 min the reaction was washed with excess 1N HCl and the organic layer was dried over MgSO<sub>4</sub> 60

and stripped to yield 37 g of 2-nitro-4-t-butyl phenol. This nitrophenol (37 g, 0.19 mole) was dissolved in 100 mL ethyl acetate and placed into a Parr bottle with a teaspoon of 10% Pd/C. The mixture was placed on a hydrogenator under 50 psi hydrogen with agitation for 1 hr. The catalyst was filtered off through celite, and the ethyl acetate was stripped off under vacuum. The material crystallized with the addition of about 200 mL heptane to give 25.6 g of the corresponding amine (2-amino-4-t-butyl phenol).

Malononitrile (39.6 g, 0.6 mole) was dissolved in methanol (38 g, 1.2 mole, 48 mL) and 200 mL of methyl formate in a 1-L, 3-neck round-bottomed flask with an ice bath and

5 with nitrogen purge and containing dimethylamino pyridine (3.8 g, 0.031 mole) and 150 mL methylene chloride. The was treated with DBU (14.1 g, 0.093 mole), stirred for 4 hr, diluted with ethyl acetate, and washed with excess 1N HCl and water. The organic layer was dried over  $MgSO_4$  and concentrated to a crude oil that was chromatographed on silica gel using methylene chloride/heptane/ethyl acetate (5/3/2) as the eluent. About 20.5 g of the inventive coupler 10 was obtained as a foam.

10



addition funnel. The mixture was cooled to 10° C. and treated dropwise over 5 min with thionyl chloride (55 g, 0.46 mole, 33.6 mL). A precipitate formed after 30 min and an additional 100 mL of methyl formate was added. After 1 hr the precipitate was collected and air dried for 20 min to yield 52 g of the corresponding imine salt intermediate 14. This salt was stored in an air-tight bottle purged with nitrogen. This imine salt (10.7 g, 0.08 mole) and 2-amino-4-t-butyl phenol (6.6 g, 0.04 mole) were heated with 100 mL methanol at 60° C. for 10 min before diluting with 200 mL of ethyl acetate and excess water. The organic layer was dried over  $MgSO_4$  and stripped to yield 8.6 g of the benzoxazole 15. This oil (4.5 g, 0.02 mole) and aldehyde DMBA (6.7 g, 0.02 mole) in 80 mL acetic acid and 3 drops of triethylamine were heated to 80° C. for 15 min and then stirred overnight at room temperature to give a slurry of crystals. The crystals were collected and washed with 100 mL methanol to give two crops yielding about 7 g of the methine dye 16. This dye (3.5 g, 0.0068 mole) was dissolved in about 25 mL methylene chloride and 2,6-lutidine (1.9 g, 0.017 mole). The mixture was treated with phosgene (1.93M in toluene, 0.014 mole, 7.2 mL) over a 1 min interval. After 10 min the mixture was washed in a separatory funnel with excess cold 1N HCl, and then with cold water. The organic phase was dried over  $MgSO_4$  and stripped to yield 3.7 g of the carbamoyl chloride 13. After scale-up, this carbamoyl chloride (17.9 g, 0.031 mole) was reacted with coupler 12 (29.3 g, 0.131 mole) in a 1-L, 3-neck round-bottomed flask fitted

Scheme II

-continued



## Photographic Examples

## EXAMPLE 1

The invention is described by the following results from a monochrome coating experiment in which the image couplers Comp-1 (check), and Inv-77 and Inv-99

(Invention) were coated with two emulsions, Emulsion A (a 15 mole percent iodide, 2.1 micrometer, saturated iodide core, silver bromoiodide emulsion) and Emulsion B (a 15 mole percent iodide, 2.1 micrometer, saturated iodide core, 5 silver bromoiodide emulsion). The emulsions were of a similar grain size but addenda were added to Emulsion B during finishing to attain a low density in the non-exposure areas (Dmin). The high dye yield image couplers, Inv-77 and Inv-99, were coated at half the molar level of comparative 10 Comp-1 conventional coupler.

The coating format for the monochrome yellow format 15 coated on Remjet film-base was as follows:

- Layer 1—Emulsion layer containing:  
 Silver bromoiodide, 15 mole % I, 1.29 g/m<sup>2</sup> Ag  
 20 Conventional image coupler Comp-1 at 0.36mM/m<sup>2</sup> or high dye-yield coupler at 0.18 mM/m<sup>2</sup>  
 Gelatin 2.69 g/m<sup>2</sup>, and spreading agents, 1.0 wt % of melt weight.
- Layer 2—Overcoat layer containing:  
 25 Gelatin 1.29 g/m<sup>2</sup>, 1,1'-(methylenebis-sulfonyl)bis-ethene hardener 1.75% of total gelatin, and spreading agents, 1.0 wt % of melt weight.

The high dye-yield imaging couplers were provided as a 30 dispersion in d-n-butyl phthalate in a weight ratio of 2:1. The conventional imaging coupler Comp-1 was provided as a dispersion without a permanent coupler solvent. The formulas for the tested couplers were as follows:



| COUPLER | X |
|---------|---|
| Comp-1  |   |
| I-77    |   |

-continued



## COUPLER

## X

I-99



Coatings were exposed to blue light through a graduated density step-wedge and processed using the Kodak Flexi-color C-41 protocol. In some cases the samples were subjected to the conventional 3.25 minute development while in others, the development time was 4.5 minutes. Sensitometric parameters were obtained from the coatings for Comp-1 for the different emulsions A and B and the contrast determined using 3.25 and 4.5 minute development times and the results are tabulated in Table I.

TABLE IA

| Coating Number | Coupler | Emulsion | Contrast 3.25 min | Contrast 4.5 min | Contrast Ratio |
|----------------|---------|----------|-------------------|------------------|----------------|
| 1              | Comp-1  | A        | 0.41              | 0.44             | 1.07           |
| 4              | Comp-1  | B        | 0.32              | 0.41             | 1.28           |

The foregoing results represent an application of the test described in the specification to identify a "low developability" emulsion. As can be seen, emulsion B exhibits a contrast ratio of at least 1.1 (a 10% increase after the longer development time) and is therefore a "low developability" emulsion. On the other hand, Emulsion A is not a "low developability" emulsion, and exhibits a Contrast Ratio of only 1.07.

A third emulsion "C" was prepared to have similar size, morphology and sensitization to the emulsion used in the inventive examples of Mooberry et al. U.S. Pat. No. 4,840,884, and was coated in the above format and subjected to the test for low developability. The results are shown in Table IB:

TABLE IB

| Coating Number | Coupler | Emulsion | Contrast 3.25 min | Contrast 4.5 min | Contrast Ratio |
|----------------|---------|----------|-------------------|------------------|----------------|
| 7              | Comp-1  | C        | 0.36              | 0.32             | 0.89           |

Coating 7 did not exhibit a ratio of at least 1.10 and was therefore not a "low developability" emulsion. Thus, the coating of the Mooberry patent was not of the type described in this specification.

As the results in Table IC show, when the inventive couplers I-77 and I-99 were coated with the check emulsion

(A) the contrast ratio showed that emulsion/coupler combination to result in a much lower contrast (ratio was 0.70 and 0.53). This was not the case for the combination of the low developability emulsion (B) and the inventive couplers where the contrast ratio was close to unity. This indicates that advantageous consistent development was obtained over a time of development range.

TABLE IC

| Coating Number | Type | Coupler | Emulsion | Contrast 3.25 min | Contrast 4.5 min | Contrast Ratio |
|----------------|------|---------|----------|-------------------|------------------|----------------|
| 1              | Comp | Comp-1  | A        | 0.41              | 0.44             | 1.07           |
| 2              | Comp | I-77    | A        | 0.47              | 0.33             | 0.70           |
| 3              | Comp | I-99    | A        | 0.38              | 0.20             | 0.53           |
| 4              | Comp | Comp-1  | B        | 0.32              | 0.41             | 1.28           |
| 5              | Inv  | I-77    | B        | 0.47              | 0.46             | 0.98           |
| 6              | Inv  | I-99    | B        | 0.47              | 0.46             | 0.98           |

In the following table, Speed refers to the exposure level on the D/logE curve where the density above D<sub>min</sub> is 20% of the average gradient from the exposure at D<sub>min</sub> to an exposure of 0.61 log E greater than D<sub>min</sub>. Inertial speed is the exposure level determined by the point where the line representing the maximum slope of the D/logE curve intersects the D<sub>min</sub> density line. Contrast is the maximum instantaneous slope of the D/logE curve.

TABLE II

| Coating Number | Coupler | Emulsion | Silver Level          | Speed ΔlogE D <sub>min</sub> vs 4 | Inertial Speed ΔlogE vs 4 | Contrast γ |
|----------------|---------|----------|-----------------------|-----------------------------------|---------------------------|------------|
| 1              | Comp-1  | A        | 1.29 g/m <sup>2</sup> | 0.13 +.01                         | 0                         | 0.42       |
| 2              | I-77    | A        | 1.29 g/m <sup>2</sup> | 0.27 +.09                         | +.12                      | 0.43       |
| 3              | I-99    | A        | 1.29 g/m <sup>2</sup> | 0.33 +.133                        | +.10                      | 0.39       |
| 4              | Comp-1  | B        | 1.29 g/m <sup>2</sup> | 0.08 —                            | —                         | 0.32       |
| 5              | I-77    | B        | 1.29 g/m <sup>2</sup> | 0.16 +.122                        | +.20                      | 0.42       |
| 6              | I-99    | B        | 1.29 g/m <sup>2</sup> | 0.18 +.09                         | +.16                      | 0.42       |

B - Finished to low D<sub>min</sub>

A comparison of coatings 1 and 4 (low D<sub>min</sub>) shows that their speed was matched but the contrast of Coating 1 was considerably higher (by 31%). The D<sub>min</sub> of coating 4 was 0.05 lower than that of coating 1. These data illustrate the

differences between the two emulsions when coated with the same conventional imaging coupler. The emulsion B has lower  $D_{min}$  and lower contrast.

Coatings 5 and 6 showed equivalent contrast to coating 1, with a very modest increase in  $D_{min}$ . More importantly, there was a significant speed increase which is a very desirable result, and that more than offsets the rise in  $D_{min}$ . Thus the high dye-yield coupler of the invention, when used in conjunction with Emulsion B, achieved a speed point considerably higher than the conventional system with only a small increase in  $D_{min}$ .

When the high dye yield couplers of the invention were combined with the more developable, more highly finished Emulsion A, in coatings 2 and 3, the speeds increased over coating 1 (but not as much as for coatings 5 and 6) while achieving equivalent contrasts, but the  $D_{min}$  values were also very much higher. This illustrates the improvement made by using the less developable Emulsion B in conjunction with the high dye yield coupler.

In other words, coatings 5 and 6 closely match coating 1 in  $D_{min}$  and gamma but show a two level improvement in speed.

In further experimentation, it was observed that the use of the inventive couplers in combination with the low developability emulsion gave the extra speed without increasing the granularity measured in the  $D_{min}$  area. This is seen in Table III comparing the rms granularities ( $\sigma D$ ) in the  $D_{min}$  areas for coatings 1, 5, and 6.

TABLE III

| Coating Number | Coupler | Emulsion | $\sigma D_{min}$ |
|----------------|---------|----------|------------------|
| 1              | Comp-1  | A        | 0.0229           |
| 2              | I-77    | A        | 0.0273           |
| 3              | I-99    | A        | 0.039            |
| 4              | Comp-1  | B        | 0.0162           |
| 5              | I-77    | B        | 0.0227           |
| 6              | I-99    | B        | 0.0331           |

The preceding examples are set forth to illustrate specific embodiments of this invention and are not intended to limit the scope of the materials or combinations of this invention. Additional embodiments and advantages within the scope of the claimed invention will be apparent to one skilled in the art. All previously cited patents, publications, and cofiled and copending patent applications are incorporated herein by reference in their entirety.

What is claimed is:

1. A photographic element comprising a support bearing at least one photographic silver halide emulsion having associated therewith at least one high dye-yield coupler that forms a first colored dye and releases from the coupling position a second dye or dye precursor having an electrically neutral dye chromophore, said second dye being in the same color range as said first dye, said emulsion exhibiting low developability.

2. The element of claim 1 wherein the high dye-yield coupler is capable of reacting with oxidized color developer to form a yellow dye.

3. The element of claim 1 wherein said high dye-yield coupler is one which releases a dye (or dye precursor) that contains a methine, azamethine, or azo group.

4. The element of claim 1 wherein said high dye-yield coupler is one wherein the released dye or dye formed from the precursor is yellow in color.

5. The element of claim 1 wherein the released dye or dye formed from the precursor has an electrically neutral dye

chromophore bonded to a linking group selected from the group consisting of  $—OC(O)—$ ,  $—OC(S)—$ ,  $—SC(O)—$ ,  $—SC(S)—$ , and  $—OC(=NSO_2R) —$  where R is a substituted or unsubstituted alkyl or aryl group.

5 6. The element of claim 1 wherein the high dye-yield coupler has the formula:



15 where COUP is the parent group of the coupler capable of reacting at the coupling position with oxidized color developer to form a first dye, T is one or more optional timing groups with m=0 to 2, L is a linking group, and DYE is a second dye.

20 7. The element of claim 6 wherein L is selected from the group consisting of  $—OC(O)—$ ,  $—OC(S)—$ ,  $—SC(O)—$ ,  $—SC(S)—$ , and  $—OC(=NSO_2R) —$  where R is a substituted or unsubstituted alkyl or aryl group.

25 8. The element of claim 6 wherein m is 1 or 2 and at least one T independently has a bond from COUP or another timing group to an oxygen atom which is bonded to a substituted or unsubstituted aromatic hydrocarbyl or heterocyclic ring at a location in conjugation with a methyl group on the ring which may optionally be substituted with one or two alkyl groups, where the methyl group is bonded to L—DYE or a second timing group.

30 9. The element of claim 6 wherein at least one T has the formula:



40 45 50 55 wherein Z is selected from the group consisting of nitro, cyano, alkylsulfonyl; sulfamoyl ( $—SO_2NR_2$ ); and sulfamido ( $—NRSO_2R$ ) groups; R is hydrogen or a substituent; R<sup>1</sup>, R<sup>11</sup> and R<sup>12</sup> are independently hydrogen or substituents that do not adversely affect the coupling and release reactions or the properties of the dyes formed thereby.

60 65 10. The element of claim 6 wherein COUP is an open chain ketomethylene compound capable of forming a yellow dye upon reaction with oxidized developer.

11. The element of claim 6 wherein DYE or the dye formed by DYE when DYE is a dye precursor is selected from I, II, and III:

I. Azo dye moieties represented by the structure:



wherein R<sup>25</sup> is hydrogen or a substituent, such as alkyl and R<sup>26</sup> and R<sup>27</sup> independently represent hydrogen or one or more substituents;

II. Azamethine dye moieties represented by the structure:



wherein R<sup>28</sup> is hydrogen or one or more substituents, such as alkyl; R<sup>29</sup> is hydrogen or a substituent, and EWG is an electron withdrawing group;

III. Methine dye moieties represented by the structure:



wherein R<sup>30</sup> and R<sup>31</sup> are independently hydrogen or a substituent, R<sup>30a</sup> is hydrogen or one or more substituents; and EWG is an electron withdrawing group having a positive Hammett's sigma(para) value.

12. The element of claim 1 wherein said emulsion has a silver iodide content of at least 6 mole percent of the total silver halide present in the layer and wherein the emulsion has a mean grain size of at least 1.5 micrometers.

13. The element of claim 6 wherein said emulsion has a silver iodide content of at least 6 mole percent of the total silver halide present in the layer and wherein the emulsion has a mean grain size of at least 1.5 micrometers.

\* \* \* \* \*